

# UNITED STATES PATENT OFFICE.

WALTHER NERNST, OF GÖTTINGEN, GERMANY, ASSIGNOR TO NERNST LAMP COMPANY, A CORPORATION OF PENNSYLVANIA.

## ELECTRIC GLOW-LAMP.

1,106,960.

Specification of Letters Patent. Patented Aug. 11, 1914.

No Drawing. Original application filed March 29, 1898, Serial No. 675,603. Divided and this application filed September 10, 1908. Serial No. 452,485.

*To all whom it may concern:*

Be it known that I, WALTHER NERNST, a subject of the German Emperor, and resident of Göttingen, in the Kingdom of Prussia, German Empire, have invented certain new and useful Improvements in Electric Glow-Lamps, of which the following is a specification.

My invention relates to the class of electric lamps in which the light emitting element or member is a non-conductor at ordinary temperatures and which may be made conductive by subjecting it to a relatively high degree of heat.

15 The object of my invention is to provide a light emitting member or glower of such composition of materials as shall specially adapt it for efficient service and long life.

I have found that a glower formed of a mixture of certain materials will become conductive at a lower temperature and be more durable in service than a glower made of a single material, provided the materials are thoroughly powdered and mixed together, then combined with a suitable binding material, and formed into the proper shape and thoroughly baked, suitable terminals of conducting material being attached to the ends of the glower in order to facilitate connecting it in circuit for operation.

30 My invention contemplates the employment of any one of a considerable variety of mixtures of materials, but mixtures of two or more of the oxids of zirconium, yttrium, thorium, beryllium, and magnesium will generally be found most desirable. I may, however, combine one of these oxids, such, for example, as the oxid of magnesium, with a small percentage of boric acid, chlorid of calcium, tungstic acid, or the like.

When a glower formed of a proper mixture of two or more of the materials above specified is connected in an electric circuit

and heated to its conducting temperature, the heat developed in itself by the passage 45 of a current therethrough will serve to maintain it in a conducting condition and cause it to yield light in a very efficient manner.

This application is a division of application, Serial No. 675,603, filed March 29, 1898, which has issued as Patent No. 900,416, and other divisions thereof are Serial No. 348,567, which has issued as Patent No. 1,071,649, and Serial No. 763,184, filed September 24, 1913.

I claim as my invention:

1. A conductor for electric lamps, consisting of an intimate mixture of yttria and tungstic acid.

2. A light giving body for electric glow lamps which is non-conductive at atmospheric temperatures and is conductive at high temperatures, consisting of an intimate mixture containing yttria and a small percentage of tungstic acid.

3. A light giving body for electric glow lamps which is non-conductive at atmospheric temperatures and is conductive at high temperatures, consisting of an intimate 70 mixture of the oxid of yttrium and the oxid of tungsten, the former greatly preponderating in quantity.

4. A glower for incandescent electric lamps, which is non-conductive at atmospheric temperatures and conductive at high temperatures, consisting of an intimate mixture of yttria and a relatively small proportion of tungstic acid formed into the desired shape and thoroughly baked.

Signed at Berlin, Germany, this 28th day of August, A. D. 1908.

WALTHER NERNST.

Witnesses:

HENRY HASPER,  
WOLDEMAR HAUPT.